



US011555159B2

(12) **United States Patent**  
**Susukida et al.**

(10) **Patent No.:** **US 11,555,159 B2**  
(b4) **Date of Patent:** **\*Jan. 17, 2023**

(54) **LUBRICATING OIL COMPOSITION**(71) Applicant: **ENEOS Corporation**, Tokyo (JP)(72) Inventors: **Yohei Susukida**, Tokyo (JP); **Yasushi Onumata**, Tokyo (JP); **Akira Tada**, Tokyo (JP); **Noriko Ayame**, Tokyo (JP)(73) Assignee: **ENEOS CORPORATION**, Tokyo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **17/290,496**(22) PCT Filed: **Nov. 6, 2019**(86) PCT No.: **PCT/JP2019/043568**

§ 371 (c)(1),

(2) Date: **Apr. 30, 2021**(87) PCT Pub. No.: **WO2020/095969**PCT Pub. Date: **May 14, 2020**(65) **Prior Publication Data**

US 2022/0002631 A1 Jan. 6, 2022

(30) **Foreign Application Priority Data**

|                         |               |
|-------------------------|---------------|
| Nov. 6, 2018 (JP) ..... | JP2018-209255 |
| Nov. 6, 2018 (JP) ..... | JP2018-209266 |
| Nov. 6, 2018 (JP) ..... | JP2018-209267 |

(51) **Int. Cl.**

|                    |           |
|--------------------|-----------|
| <b>C10M 141/10</b> | (2006.01) |
| <b>C10M 169/04</b> | (2006.01) |
| <b>C10M 129/54</b> | (2006.01) |
| <b>C10M 133/12</b> | (2006.01) |
| <b>C10M 133/44</b> | (2006.01) |
| <b>C10M 135/10</b> | (2006.01) |
| <b>C10M 137/02</b> | (2006.01) |
| <b>C10M 139/00</b> | (2006.01) |
| <b>C10M 177/00</b> | (2006.01) |
| <b>C10N 40/00</b>  | (2006.01) |

(Continued)

(52) **U.S. Cl.**

|           |                                                                                                                                                                                                                                                                                                                                                                                                                                                                                                                                                                                                                                                                                     |
|-----------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| CPC ..... | <b>C10M 141/10</b> (2013.01); <b>C10M 129/54</b> (2013.01); <b>C10M 133/12</b> (2013.01); <b>C10M 133/44</b> (2013.01); <b>C10M 135/10</b> (2013.01); <b>C10M 137/02</b> (2013.01); <b>C10M 139/00</b> (2013.01); <b>C10M 169/04</b> (2013.01); <b>C10M 177/00</b> (2013.01); <b>C10M 2203/003</b> (2013.01); <b>C10M 2207/144</b> (2013.01); <b>C10M 2215/26</b> (2013.01); <b>C10M 2215/30</b> (2013.01); <b>C10M 2219/044</b> (2013.01); <b>C10M 2223/049</b> (2013.01); <b>C10M 2227/061</b> (2013.01); <b>C10N 2030/02</b> (2013.01); <b>C10N 2030/04</b> (2013.01); <b>C10N 2030/041</b> (2020.05); <b>C10N 2030/10</b> (2013.01); <b>C10N 2030/14</b> (2013.01); <b>C10N</b> |
|-----------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|

2030/42 (2020.05); **C10N 2040/04** (2013.01); **C10N 2040/25** (2013.01); **C10N 2040/40** (2020.05); **C10N 2070/00** (2013.01)

(58) **Field of Classification Search**

|            |                                                                                                            |
|------------|------------------------------------------------------------------------------------------------------------|
| CPC .....  | <b>C10N 2030/14</b> ; <b>C10N 2040/40</b> ; <b>C10M 169/04</b> ; <b>C10M 133/44</b> ; <b>C10M 2215/153</b> |
| USPC ..... | <b>508/279</b> , <b>291</b>                                                                                |

See application file for complete search history.

(56) **References Cited**

## U.S. PATENT DOCUMENTS

|               |         |                  |                    |
|---------------|---------|------------------|--------------------|
| 5,840,663 A * | 11/1998 | Nibert .....     | <b>C10M 141/10</b> |
|               |         |                  | 508/279            |
| 6,103,673 A   | 8/2000  | Sumiejski et al. |                    |

(Continued)

## FOREIGN PATENT DOCUMENTS

|    |           |        |
|----|-----------|--------|
| CN | 104845706 | 8/2015 |
| EP | 0987311   | 3/2000 |

(Continued)

## OTHER PUBLICATIONS

ISR issued in WIPO Patent Application No. PCT/JP2019/043568, Feb. 10, 2020, English translation.

(Continued)

Primary Examiner — Ellen M McAvoy

(74) Attorney, Agent, or Firm — Greenblum &amp; Bernstein, P.L.C.

(57) **ABSTRACT**

A lubricating oil composition including: a lubricant base oil; (A) a triazole metal deactivator in an amount of 0.005 to 0.03 mass % in terms of nitrogen on the basis of the total mass of the composition; and (B1) a succinimide compound represented by the following general formula (1) in an amount of 0.0005 to 0.02 mass % in terms of nitrogen on the basis of the total mass of the composition:



wherein in the general formula (1), R<sup>1</sup> and R<sup>2</sup> each independently represent a hydrogen atom or a C1-36 linear or branched chain alkyl or alkenyl group, and at least one of R<sup>1</sup> and R<sup>2</sup> is a C8-36 linear or branched chain alkyl or alkenyl group, and n represents an integer of 1 to 10.

|                              |           |                     |              |                  |             |                 |              |
|------------------------------|-----------|---------------------|--------------|------------------|-------------|-----------------|--------------|
| (51) <b>Int. Cl.</b>         |           |                     |              |                  |             |                 |              |
| C10N 30/04                   | (2006.01) |                     |              | 2020/0332216 A1* | 10/2020     | Hamachi .....   | C10M 169/041 |
| C10N 30/02                   | (2006.01) |                     |              | 2021/0122994 A1* | 4/2021      | Fang .....      | C10M 141/10  |
| C10N 30/10                   | (2006.01) |                     |              | 2021/0395634 A1  | 12/2021     | Susukida et al. |              |
| C10N 30/14                   | (2006.01) |                     |              | 2021/0395635 A1  | 12/2021     | Susukida et al. |              |
| C10N 40/04                   | (2006.01) |                     |              | 2022/0025292 A1* | 1/2022      | Tamura .....    | H01M 10/613  |
| C10N 30/00                   | (2006.01) |                     |              |                  |             |                 |              |
| C10N 40/25                   | (2006.01) |                     |              |                  |             |                 |              |
| C10N 70/00                   | (2006.01) |                     |              |                  |             |                 |              |
| (56) <b>References Cited</b> |           |                     |              |                  |             |                 |              |
| U.S. PATENT DOCUMENTS        |           |                     |              |                  |             |                 |              |
| 8,987,178 B2 *               | 3/2015    | Davies .....        | C10M 159/20  | JP               | 09-202890   | 8/1997          |              |
|                              |           |                     | 508/574      | JP               | 09-328698   | 12/1997         |              |
| 2002/0010102 A1*             | 1/2002    | Koshima .....       | C07F 9/4006  | JP               | 11-171892   | 6/1999          |              |
|                              |           |                     | 508/432      | JP               | 2000-087068 | 3/2000          |              |
| 2004/0192562 A1              | 9/2004    | Morita et al.       |              | JP               | 2003-113391 | 4/2003          |              |
| 2004/0209786 A1              | 10/2004   | Sagawa et al.       |              | JP               | 2005-325355 | 11/2005         |              |
| 2005/0250656 A1              | 11/2005   | Ishikawa et al.     |              | JP               | 2008-285682 | 11/2008         |              |
| 2008/0058233 A1              | 3/2008    | Sagawa et al.       |              | JP               | 2010-530470 | 9/2010          |              |
| 2008/0110799 A1              | 5/2008    | Matsui et al.       |              | JP               | 2011-046938 | 3/2011          |              |
| 2010/0130390 A1              | 5/2010    | Tipton et al.       |              | JP               | 2012-207083 | 10/2012         |              |
| 2010/0137173 A1*             | 6/2010    | Sheets .....        | C07D 207/412 | JP               | 2016-108406 | 6/2016          |              |
|                              |           |                     | 508/192      | JP               | 2016-190953 | 11/2016         |              |
| 2010/0317554 A1              | 12/2010   | Fuchi et al.        |              | JP               | 2018-053017 | 4/2018          |              |
| 2011/0028364 A1*             | 2/2011    | Shrestha .....      | C10M 133/16  | WO               | 2007/052826 | 5/2007          |              |
|                              |           |                     | 508/291      |                  |             |                 |              |
| 2012/0090568 A1              | 4/2012    | Teshima et al.      |              |                  |             |                 |              |
| 2014/0018271 A1*             | 1/2014    | Onumata .....       | C10M 141/10  |                  |             |                 |              |
|                              |           |                     | 508/433      |                  |             |                 |              |
| 2016/0108337 A1*             | 4/2016    | Abraham .....       | C10M 145/14  |                  |             |                 |              |
|                              |           |                     | 508/162      |                  |             |                 |              |
| 2017/0204046 A1              | 7/2017    | Kishi et al.        |              |                  |             |                 |              |
| 2018/0087002 A1              | 3/2018    | Komatsubara et al.  |              |                  |             |                 |              |
| 2018/0100117 A1*             | 4/2018    | Flores-Torres ..... | C10M 167/00  |                  |             |                 |              |
| 2018/0100118 A1*             | 4/2018    | Flores-Torres ..... | C10M 169/04  |                  |             |                 |              |

## FOREIGN PATENT DOCUMENTS

|    |             |         |
|----|-------------|---------|
| JP | 09-202890   | 8/1997  |
| JP | 09-328698   | 12/1997 |
| JP | 11-171892   | 6/1999  |
| JP | 2000-087068 | 3/2000  |
| JP | 2003-113391 | 4/2003  |
| JP | 2005-325355 | 11/2005 |
| JP | 2008-285682 | 11/2008 |
| JP | 2010-530470 | 9/2010  |
| JP | 2011-046938 | 3/2011  |
| JP | 2012-207083 | 10/2012 |
| JP | 2016-108406 | 6/2016  |
| JP | 2016-190953 | 11/2016 |
| JP | 2018-053017 | 4/2018  |
| WO | 2007/052826 | 5/2007  |

## OTHER PUBLICATIONS

IPRP issued in WIPO Patent Application No. PCT/JP2019/043568, May 11, 2021, English translation.  
 ISR of PCT/JP2019/043567, Feb. 10, 2020, translation.  
 IPRP of PCT/JP2019/043567, May 11, 2021, translation.  
 ISR of PCT/JP2019/043569, Feb. 10, 2020, translation.  
 IPRP of PCT/JP2019/043569, May 11, 2021, translation.  
 U.S. OA issued in U.S. Appl. No. 17/289,961, filed Oct. 26, 2021.  
 U.S. OA issued in U.S. Appl. No. 17/289,993, filed Nov. 2, 2021  
 U.S. final Office Action issued in U.S. Appl. No. 17/289,993, dated Mar. 10, 2022.  
 U.S. Office Action issued in U.S. Appl. No. 17/289,961, dated Aug. 8, 2022.

\* cited by examiner

**1**  
**LUBRICATING OIL COMPOSITION**

**FIELD**

The present invention relates to a lubricating oil composition, and specifically to a lubricating oil composition suitable for lubrication of electric motors.

**BACKGROUND**

In recent years, electric vehicles which use an electric motor as a power source for running, and hybrid vehicles which use an electric motor and an internal combustion engine together as a power source for running are attracting interest in view of energy efficiency and environmental compatibility. While generating heat during operation thereof, electric motors include heat-sensitive components such as a coil and a magnet. Those vehicles using an electric motor as a power source for running are thus provided with means for cooling the electric motor. Known means for cooling the electric motor include air cooling, water cooling and oil cooling. Among them, oil cooling is to circulate oil in the electric motor, to directly make parts in the electric motor which generate heat (such as a coil, a core and a magnet) contact with a coolant (oil), which makes it possible to obtain a high cooling effect. In the electric motor using oil cooling, oil (lubricating oil) is circulated in the electric motor, to cool and lubricate the electric motor at the same time. Electrical insulation, and corrosion inhibition performance for copper used as a material of the electric motor are required of a lubricating oil (electric motor oil) of the electric motor.

The vehicle using the electric motor as a power source for running usually includes a transmission having a gear mechanism. Various additives are incorporated into a lubricating oil to lubricate the gear mechanism since anti-wear performance and anti-fatigue performance are required of the lubricating oil.

**CITATION LIST**

**Patent Literature**

- [Patent Literature 1] JP 2003-113391 A
- [Patent Literature 2] JP H9-328698 A
- [Patent Literature 3] JP 2018-053017 A

**SUMMARY**

**Technical Problem**

A lubricating oil used for lubricating the electric motor is usually different from that used for lubricating the transmission. If the electric motor and the transmission (gear mechanism) can be lubricated using the same lubricating oil, a lubricating oil circulation system can be simplified. Recently, an electric drive module into which an electric motor and a transmission (gear mechanism) are integrated as one device (package) has been also proposed. For lubrication of such an electric drive module, it is desirable to lubricate the electric motor and the transmission (gear mechanism) using the same lubricating oil in view of downsizing and weight reduction.

Disadvantageously, conventional transmission oils suffer insufficient long-term stability of electrical insulation and copper corrosion inhibition performance when they are oxidatively deteriorated by the use thereof even if electrical

**2**

insulation and copper corrosion inhibition performance of fresh oils thereof are improved for the use for lubrication of the electric motor.

An object of the present invention is to provide a lubricating oil composition having improved long-term stability of electrical insulation and copper corrosion inhibition performance after the composition is oxidatively deteriorated.

**Solution to Problem**

The present invention encompasses the following embodiments [1] to [17].

[1] A lubricating oil composition comprising:  
a lubricant base oil;

(A) a triazole metal deactivator in an amount of 0.005 to 0.03 mass % in terms of nitrogen on the basis of the total mass of the composition; and

(B1) a succinimide compound represented by the following general formula (1) in an amount of 0.0005 to 0.02 mass % in terms of nitrogen on the basis of the total mass of the composition:



wherein in the general formula (1), R<sup>1</sup> and R<sup>2</sup> each independently represent a hydrogen atom or a C1-36 linear or branched chain alkyl or alkenyl group, and at least one of R<sup>1</sup> and R<sup>2</sup> is a C8-36 linear or branched chain alkyl or alkenyl group, and n represents an integer of 1 to 10.

[2] The lubricating oil composition according to [1], further comprising:

(C) a calcium salicylate detergent in an amount of 0.005 to 0.03 mass % in terms of calcium on the basis of the total mass of the composition.

[3] The lubricating oil composition according to [1] or [2], wherein a total content of any metallic detergent is 0.005 to 0.03 mass % in terms of metal on the basis of the total mass of the composition.

[4] The lubricating oil composition according to any one of [1] to [3], wherein a proportion of any salicylate in a total soap group content of any metallic detergent is no less than 65 mass %.

[5] The lubricating oil composition according to any one of [1] to [4], further comprising:

(D) a phosphite ester compound represented by the following general formula (3) in an amount of 0.01 to 0.06 mass % in terms of phosphorus on the basis of the total mass of the composition:



wherein in the general formula (3), R<sup>4</sup> and R<sup>5</sup> are each independently a C1-18 linear chain hydrocarbon group, or a C4-20 group represented by the following general formula (4):



wherein in the general formula (4), R<sup>6</sup> is a C2-17 linear chain hydrocarbon group, and R<sup>7</sup> is a C2-17 linear chain hydrocarbon group, and X<sup>1</sup> is an oxygen atom or a sulfur atom.

[6] The lubricating oil composition according to any one of [1] to [5], optionally further comprising:

(E) a succinimide ashless dispersant in an amount of no more than 10 mass % on the basis of the total mass of the composition,

the component (E) being a first condensation reaction product, or a derivative thereof, or any combination thereof,

the first condensation reaction product being a condensation reaction product of a first alkyl- or alkenyl-succinic acid or anhydride thereof and a polyamine,

the first alkyl- or alkenyl-succinic acid having a C40-400 alkyl or alkenyl group.

[7] The lubricating oil composition according to any one of [1] to [6],

the component (B1) being a second condensation reaction product,

the second condensation product being a condensation reaction product of a second alkyl- or alkenyl-succinic acid or anhydride thereof and a polyamine,

the second alkyl- or alkenyl-succinic acid having a C8-30 alkyl or alkenyl group.

[8] The lubricating oil composition according to any one of [1] to [7],

wherein the composition has a kinematic viscosity at 40° C. of 4 to 20 mm<sup>2</sup>/s; and

the composition has a kinematic viscosity at 100° C. of 1.8 to 4.0 mm<sup>2</sup>/s.

[9] The lubricating oil composition according to any one of [1] to [8], optionally further comprising:

an amine antioxidant as (F) an antioxidant in an amount of no more than 0.15 mass % in terms of nitrogen on the basis of the total mass of the composition.

[10] The lubricating oil composition according to any one of [1] to [9], wherein a total content of (B) a nitrogen-containing oiliness agent-based friction modifier is no more than 0.03 mass % in terms of nitrogen on the basis of the total mass of the composition, a content of the component (B) being a total content of any aliphatic amine compound having a C8-36 aliphatic hydrocarbyl group other than a succinimide ashless dispersant and an amine antioxidant, and any compound having a C8-36 aliphatic hydrocarbyl or aliphatic hydrocarbylcarbonyl group and an amide bond other than a succinimide ashless dispersant and an amine antioxidant.

[11] The lubricating oil composition according to any one of [1] to [10], wherein a total phosphorus content in the lubricating oil composition is no more than 0.06 mass % in terms of phosphorus on the basis of the total mass of the composition.

[12] The lubricating oil composition according to any one of [1] to [11], wherein a total content of any metal element

in the lubricating oil composition is no more than 0.03 mass % in terms of metal on the basis of the total mass of the composition.

[13] The lubricating oil composition according to any one of [1] to [12], wherein a total content of any compound having an O/N-based active hydrogen compound is 0 to 500 mass ppm in terms of the sum of oxygen content and nitrogen content on the basis of the total mass of the lubricating oil composition, the compound not contributing to any content of the metallic detergent, the succinimide ashless dispersant, the amine antioxidant, the component (B1), a phosphite diester compound that does not have an O/N-based active hydrogen-containing group in its alcohol residue, and a triazole metal deactivator, the O/N-based active hydrogen-containing group representing a non-phenolic OH group that may be part of any other functional group, or a salt thereof, >NH group, or —NH<sub>2</sub> group.

[14] The lubricating oil composition according to any one of [1] to [13], wherein an oxidatively deteriorated oil of the composition has a volume resistivity at 80° C. of no less than 1.0×10<sup>9</sup> Ω·cm, wherein the oxidatively deteriorated oil is obtained by oxidatively treating the composition for 150 hours by ISOT method conforming to JIS K2514-1.

[15] The lubricating oil composition according to any one of [1] to [14], wherein the composition is used to lubricate an electric motor or to lubricate the electric motor and a transmission, in an automobile comprising the electric motor.

[16] A method for lubricating an electric motor, the method comprising: lubricating an electric motor installed in an automobile, by means of the lubricating oil composition as defined in any one of [1] to [15].

[17] A method for lubricating an electric motor and a transmission, the method comprising: lubricating an electric motor and a transmission installed in an automobile, by means of the lubricating oil composition as defined in any one of [1] to [15].

#### Advantageous Effects

According to the first aspect of the present invention, a lubricating oil composition having improved long-term stability of electrical insulation and copper corrosion inhibition performance after the composition is oxidatively deteriorated can be provided.

The lubricating oil composition according to the first aspect of the present invention may be preferably used for the lubricating method according to the second aspect of the present invention.

#### DESCRIPTION OF EMBODIMENTS

The present invention will be hereinafter described. In the present description, expression "A to B" concerning numeral values A and B means "no less than A and no more than B" unless otherwise specified. In such expression, if a unit is added only to the numeral value B, the same unit is applied to the numeral value A. Also, a word "or" means a logical sum unless otherwise specified. In the present description, expression "E<sub>1</sub> and/or E<sub>2</sub>" concerning elements E<sub>1</sub> and E<sub>2</sub> means "E<sub>1</sub>, or E<sub>2</sub>, or the combination thereof", and expression "E<sub>1</sub>, . . . , E<sub>N-1</sub>, and/or E<sub>N</sub>" concerning elements E<sub>1</sub>, . . . , E<sub>N</sub> (N is an integer of 3 or more) means "E<sub>1</sub>, . . . , E<sub>N-1</sub>, or E<sub>N</sub>, or any combination thereof".

<Lubricating Base Oil>

As a lubricating base oil in the lubricating oil composition according to the present invention (hereinafter may be

referred to as "lubricating oil composition" or simply "composition"), at least one mineral base oil, at least one synthetic base oil, or any mixed base oil thereof may be used, and in one embodiment, a Group II base oil, a Group III base oil, a Group IV base oil, or a Group V base oil of API base stock categories, or a mixed base oil thereof may be preferably used. An API Group II base oil is a mineral base oil containing no more than 0.03 mass % sulfur and no less than 90 mass % saturates, and having a viscosity index of no less than 80 and less than 120. An API Group III base oil is a mineral base oil containing no more than 0.03 mass % sulfur and no less than 90 mass % saturates, and having a viscosity index of no less than 120. An API Group IV base oil is a poly- $\alpha$ -olefin base oil. An API Group V base oil is a base oil other than the foregoing Groups I to IV base oils, and preferred examples thereof includes ester base oils.

The mineral base oil may be, for example, a paraffinic or naphthenic mineral base oil obtained through application of one or at least two of refining means in suitable combination, such as solvent deasphalting, solvent extraction, hydrocracking, solvent dewaxing, catalytic dewaxing, hydrorefining, sulfuric acid washing, and white clay treatment, to lubricant oil fractions that are obtained by distillation of crude oil under atmospheric pressure and under reduced pressure. API Group II and Group III base oils are usually produced via hydrocracking. A wax isomerized base oil, a base oil produced by a process of isomerizing GTL WAX (gas to liquid wax), or the like may be also used.

Examples of API Group IV base oils include ethylene-propylene copolymers, polybutene, 1-octene oligomers, and 1-decene oligomers, and hydrogenated products thereof.

Examples of API Group V base oils include monoesters (such as butyl stearate, octyl laurate, and 2-ethylhexyl oleate); diesters (such as ditridecyl glutarate, bis(2-ethylhexyl) adipate, diisodecyl adipate, ditridecyl adipate, and bis(2-ethylhexyl) sebacate); polyesters (such as trimellitate esters); and polyol esters (such as trimethylolpropane caprylate, trimethylolpropane pelargonate, pentaerythritol 2-ethylhexanoate, and pentaerythritol pelargonate).

The lubricating base oil (total base oil) may comprise one base oil, or may be a mixed base oil comprising at least two base oils. In the mixed base oil comprising at least two base oils, the API base stock categories of these base oils may be the same, or may be different from each other. The content of the API Group V base oil is preferably 0 to 20 mass %, and more preferably 0 to 15 mass %; and in one embodiment, may be 0 to 10 mass %, on the basis of the total mass of the lubricating base oil. The content of the ester base oil at the above described upper limit or less can improve oxidation stability of the lubricating oil composition.

The kinematic viscosity of the lubricating base oil (total base oil) at 100° C. is preferably 1.7 to 4.0 mm<sup>2</sup>/s, and more preferably 2.2 to 3.0 mm<sup>2</sup>/s; and in one embodiment, may be 1.7 to 3.5 mm<sup>2</sup>/s. The kinematic viscosity of the lubricating base oil at 100° C. at the above described upper limit or less can improve fuel efficiency. The kinematic viscosity of the lubricating base oil at 100° C. at the above described lower limit or more can improve anti-wear performance, and anti-fatigue performance, and can also improve electrical insulation of a fresh oil. In the present description, "kinematic viscosity at 100° C." means a kinematic viscosity at 100° C. specified in ASTM D-445.

The kinematic viscosity of the lubricating base oil (total base oil) at 40° C. is preferably 5.0 to 20.0 mm<sup>2</sup>/s, and more preferably 7.0 to 12.0 mm<sup>2</sup>/s; and in one embodiment, may be 5.0 to 14.7 mm<sup>2</sup>/s. The kinematic viscosity of the lubricating base oil at 40° C. at the above described upper

limit or less can improve fuel efficiency. The kinematic viscosity of the lubricating base oil at 40° C. at the above described lower limit or more can improve anti-wear performance and anti-fatigue performance, and can also improve electrical insulation of a fresh oil. In the present description, "kinematic viscosity at 40° C." means a kinematic viscosity at 40° C. specified in ASTM D-445.

The viscosity index of the lubricating base oil (total base oil) is preferably no less than 100, and more preferably no less than 105; and in one embodiment, may be no less than 110, may be no less than 120, and may be no less than 125. The viscosity index of the lubricating base oil at the above described lower limit or more can improve viscosity-temperature characteristics and thermal and oxidation stability, can reduce a friction coefficient, and can improve anti-wear performance of the lubricating oil composition. In the present description, a viscosity index means a viscosity index measured conforming to JIS K 2283-1993.

The sulfur content in the lubricating base oil (total base oil) is, in view of oxidation stability, preferably no more than 0.03 mass % (300 mass ppm), more preferably no more than 50 mass ppm, and especially preferably no more than 10 mass ppm, and may be no more than 1 mass ppm.

The lubricating base oil (total base oil) is a major constituent of the lubricating oil composition. The content of the lubricating base oil (total base oil) in the lubricating oil composition is preferably 80 to 98 mass %, and more preferably 83 to 90 mass %; and in one embodiment, may be 83 to 93 mass %, on the basis of the total mass of the composition.

<(A) Triazole Metal Deactivator>

The lubricating oil composition according to the present invention comprises (A) a triazole metal deactivator (hereinafter may be referred to as "component (A)"). As the component (A), any tolyltriazole metal deactivator and/or benzotriazol metal deactivator used in lubricating oils may be used without particular limitations. As the component (A), one compound may be used alone, or at least two compounds may be used in combination.

The content of the component (A) in the lubricating oil composition is 0.005 to 0.03 mass % in terms of nitrogen on the basis of the total mass of the composition. The content of the component (A) at the above described lower limit or more can improve long-term stability of copper corrosion inhibition. The content of the component (A) at the above described upper limit or less can improve electrical insulation of a fresh oil and the oxidatively deteriorated composition.

<(B) Nitrogen-Containing Oiliness Agent-Based Friction

Modifier>

In one embodiment, the lubricating oil composition may comprise a nitrogen-containing oiliness agent-based friction modifier (hereinafter may be simply referred to as "component (B)"). Examples of the nitrogen-containing oiliness agent-based friction modifier include oiliness agent-based friction modifiers such as (B1) a succinimide friction modifier described later, and amine friction modifiers and amide friction modifiers. The component (B) encompasses aliphatic amine compounds each having a C8-36 aliphatic hydrocarbyl group, other than a succinimide ashless dispersant (component (E)) and an amine antioxidant (component (F)), and compounds each having a C8-36 aliphatic hydrocarbyl or aliphatic hydrocarbylcarbonyl group and an amide bond other than the succinimide ashless dispersant (component (E)) and the amine antioxidant (component (F)).

Examples of the amine friction modifier include aliphatic amine compounds each having a C10-30, preferably a

C12-24, more preferably a C12-20 alkyl or alkenyl, preferably linear chain alkyl or linear chain alkenyl group.

Examples of the amide friction modifier include condensation products of a linear or branched chain, preferably linear chain fatty acid, and ammonia, an aliphatic monoamine or an aliphatic polyamine.

One example of the amide friction modifier is a fatty acid amide compound having a C10-30, preferably a C12-24 alkylcarbonyl or alkenylcarbonyl group. For example, such an amide compound can be obtained by a condensation reaction of a C10-30, preferably a C12-24 fatty acid or an acid chloride thereof, and an aliphatic primary or secondary amine compound, an aliphatic primary or secondary alkanolamine compound, or ammonia. The foregoing amine compound and alkanolamine compound each preferably have a C1-30, more preferably a C1-10, further preferably a C1-4 aliphatic group; and in one embodiment, each have a C1 or C2 aliphatic group.

Examples of the fatty acid amide friction modifier include lauramide, myristamide, palmitamide, stearamide, oleamide, cocamide, and C12-13 synthetic mixed fatty acid amides.

Other examples of the amide friction modifier include fatty acid hydrazides, fatty acid semicarbazides, aliphatic ureas, fatty acid ureides, and aliphatic allophanamides each having a C10-30 alkyl or alkenyl group, or a C10-30 alkylcarbonyl or alkenylcarbonyl group, and derivatives (modified compounds) thereof. Examples of the derivative (modified compound) of the amide friction modifier include boric acid-modified compounds obtained by reacting any amide compound as described above with boric acid or a boric acid salt.

Examples of the aliphatic urea friction modifier include aliphatic urea compounds each having a C12-24, preferably a C12-20 alkyl or alkenyl group such as dodecylurea, tridecylurea, tetradecylurea, pentadecylurea, hexadecylurea, heptadecylurea, octadecylurea, and oleylurea, and acid-modified derivatives thereof (acid-modified compounds such as boric acid-modified compounds).

Examples of the fatty acid hydrazide friction modifier include fatty acid hydrazide compounds each having a C12-24 alkylcarbonyl or alkenylcarbonyl group, such as dodecanoic hydrazide, tridecanoic hydrazide, tetradecanoic hydrazide, pentadecanoic hydrazide, hexadecanoic hydrazide, heptadecanoic hydrazide, octadecanoic hydrazide, oleic hydrazide, erucic hydrazide, and acid-modified derivatives thereof (acid-modified compounds such as boric acid-modified compounds).

Other examples of the amide friction modifier include amide compounds of aliphatic hydroxy acids each having a C1-30 hydroxy-substituted alkyl or alkenyl group. Such an amide compound can be obtained by, for example, a condensation reaction of any aliphatic hydroxy acid as described above with an aliphatic primary or secondary amine compound, or an aliphatic primary or secondary alkanolamine compound. The carbon number of a hydroxy-substituted alkyl or alkenyl group of the above described aliphatic hydroxy acid is preferably 1 to 10, more preferably 1 to 4; and in one embodiment, 1 or 2. The aliphatic hydroxy acid is preferably a linear chain aliphatic  $\alpha$ -hydroxy acid, and in one embodiment, is a glycolic acid. The above described amine compounds and alkanolamine compounds each preferably have a C1-30, more preferably a C10-30, further preferably a C12-24, and especially preferably a C12-20 aliphatic group.

Other examples of the amide friction modifier include amide any compounds of a C10-30, preferably a C12-24

fatty acid, and an amino acid (N-acylated amino acid). Examples of the N-acylated amino acid friction modifier include N-acylated-N-methylglycine (such as N-oleoyl-N-methylglycine).

5 (B1) Succinimide Friction Modifier

The lubricating oil composition according to the present invention comprises (B1) a succinimide compound represented by the following general formula (1) (hereinafter may be referred to as a "succinimide friction modifier", or simply "component (B1)"). As the component (B1), one compound may be used alone, or at least two compounds may be used in combination.

(1)



In the general formula (1), R<sup>1</sup> and R<sup>2</sup> each independently represent a hydrogen atom, or a C1-36 linear or branched chain alkyl or alkenyl group, and at least one of R<sup>1</sup> and R<sup>2</sup> is a C8-36 linear or branched chain alkyl or alkenyl group. R<sup>1</sup> and R<sup>2</sup> are preferably C8-30, more preferably C12-24, and further preferably C12-22 linear or branched chain alkyl or alkenyl groups. n represents an integer of 1-10, preferably 1-7, more preferably 1-4, and further preferably 1-3.

The method for producing a succinimide compound that may be used as the component (B1) is not specifically limited. For example, the component (B1) may be obtained as a condensation reaction product (bisimide) by: reaction of alkyl- or alkenyl-succinic acid having a C8-36, preferably a C8-30, more preferably a C12-22 alkyl or alkenyl group, or anhydride thereof, with a polyamine. Here, examples of the polyamine include diethylenetriamine, triethylenetetramine, tetraethylenepentamine, and pentaethylenhexamine, and any mixtures thereof, and a polyamine raw material comprising at least one selected therefrom may be preferably used. The polyamine raw material may further or optionally comprise ethylenediamine. In view of improvement of the performance of the condensation product or derivative thereof as a friction modifier, the content of ethylenediamine in the polyamine raw material is preferably 0 to 10 mass %, and more preferably 0 to 5 mass %, on the basis of the total mass of the polyamine raw material.

The content of the component (B1) in the lubricating oil composition is 0.0005 to 0.02 mass %, and in one embodiment, 0.001 to 0.02 mass %, in terms of nitrogen on the basis of the total mass of the composition. The content of the component (B1) at the above described upper limit or less can improve electrical insulation of a fresh oil and the oxidatively deteriorated composition. The content of the component (B1) at the above described lower limit or more can improve long-term stability of copper corrosion inhibition performance, and can reduce a friction coefficient for a long period of time. In the present description, the content of the component (B1) shall contribute to the content of the component (B).

The lubricating oil composition may optionally comprise 65 the component (B) other than the component (B1). The total content of the component (B) in the lubricating oil composition is preferably no more than 0.03 mass %, and in one

embodiment, may be no more than 0.02 mass %, in terms of nitrogen on the basis of the total mass of the composition. The total content of the component (B) at the above described upper limit or less can further improve electrical insulation of a fresh oil and the oxidatively deteriorated composition.

<(C) Calcium Salicylate Detergent>

In one preferred embodiment, the lubricating oil composition may further comprise (C) a calcium salicylate detergent (hereinafter may be simply referred to as "component (C)"). As the component (C), a calcium salicylate, or a basic salt or overbased salt thereof may be used. As the component (C), one calcium salicylate detergent may be used alone, or at least two calcium salicylate detergents may be used in combination. Examples of the calcium salicylate include any compound represented by the following general formula (2).



In the general formula (2), R<sup>3</sup> each independently represent a C14-30 alkyl or alkenyl group; and a represents 1 or 2, and is preferably 1. The compound represented by the general formula (2) may be a mixture of any compound of the general formula (2) where a=1 and any compound of the general formula (2) where a=2. When a=2, R<sup>3</sup> may be any combination of different groups.

One preferred embodiment of the calcium salicylate detergent may be a calcium salicylate represented by a compound of the above general formula (2) where a=1, or a basic salt or overbased salt thereof.

The method for producing the calcium salicylate is not particularly restricted, and a known method for producing monoalkylsalicylates or the like may be used. For example, the calcium salicylate may be obtained by: making a calcium base such as oxides and hydroxides of calcium react with a monoalkylsalicylic acid obtained by alkylating a phenol as a starting material with an olefin, and then carboxylating the resultant product with carbonic acid gas or the like, or with a monoalkylsalicylic acid obtained by alkylating a salicylic acid as a starting material with an equivalent of the olefin, or the like; converting the above monoalkylsalicylic acid or the like to an alkali metal salt such as a sodium salt and a potassium salt, and then performing transmetallation with a calcium salt; or the like.

The method for obtaining the overbased calcium salicylate is not particularly restricted. For example, a calcium salicylate is made to react with a calcium base such as calcium hydroxide in the presence of carbonic acid gas, which makes it possible to obtain the overbased calcium salicylate.

The base number of the component (C) is not particularly limited, but is preferably 50 to 350 mgKOH/g, more preferably 100 to 350 mgKOH/g, and especially preferably 150 to 350 mgKOH/g. The base number of the component (C) at the above described lower limit or more can lead to further improved electrical insulation of the oxidatively deteriorated composition.

The content of the component (C) in the lubricating oil composition when the lubricating oil composition comprises the component (C) is preferably 0.005 to 0.03 mass %, and preferably 0.005 to 0.02 mass %, in terms of calcium on the

basis of the total mass of the lubricating oil composition. The content of the component (C) at the above described upper limit or less can further improve electrical insulation of a fresh oil and the oxidatively deteriorated composition. The content of the component (C) at the above described lower limit or more can improve anti-fatigue performance.

The lubricating oil composition may comprise the component (C) only, or may further comprise at least one metallic detergent other than the calcium salicylate detergent (such as a calcium sulfonate detergent and a calcium phenate detergent) in addition to the component (C), as a metallic detergent. The total content of the metallic detergent in the lubricating oil composition is preferably 0.005 to 0.03 mass % in terms of metal on the basis of the total mass of the composition. The total content of the metallic detergent in the lubricating oil composition at the above described upper limit or less can further improve electrical insulation of a fresh oil and the oxidatively deteriorated composition. The proportion of total salicylates in the total soap group content of the metallic detergent, that is, the proportion of mass of the total soap group of the salicylate detergent in terms of organic acid to mass of the total soap group of the metallic detergent in terms of organic acid is preferably 65 to 100 mass %, and more preferably 90 to 100 mass %. Contribution of salicylates to the total soap group content of the metallic detergent at the above described lower limit or more can improve anti-fatigue performance. In the present description, a soap group of the metallic detergent means a conjugate base of an organic acid which constitutes the soap content of the metallic detergent (examples thereof in the salicylate detergent include alkylsalicylate anions, examples thereof in the sulfonate detergent include alkylbenzenesulfonate anions, and examples thereof in the phenate detergent include alkylphenate anions).

<(D) Phosphite Ester Compound>

In one preferred embodiment, the lubricating oil composition may further comprise a phosphite ester compound (hereinafter may be referred to as "component (D)" represented by the following general formula (3). As the component (D), one phosphite ester compound may be used alone, or at least two phosphite ester compounds may be used in combination.



In the general formula (3), R<sup>4</sup> and R<sup>5</sup> are each independently a C1-18 linear chain hydrocarbon group, or a C4-20 group represented by the following general formula (4), preferably a C5-20 group represented by the general formula (10).



In the general formula (4), R<sup>6</sup> is a C2-17 linear chain hydrocarbon group, preferably an ethylene group or a propylene group, and in one embodiment, an ethylene group; R<sup>7</sup> is a C2-17, preferably a C2-16, and especially preferably a

## 11

C6-10 linear chain hydrocarbon group. X<sup>1</sup> is an oxygen atom or a sulfur atom, preferably a sulfur atom.

Using a phosphite ester compound having the foregoing structure as the component (D) can further improve anti-wear performance and anti-fatigue performance.

In one embodiment, preferred examples of R<sup>4</sup> and R<sup>5</sup> include C4-18 linear chain alkyl groups. Examples of the linear chain alkyl group include butyl group, pentyl group, hexyl group, heptyl group, octyl group, nonyl group, decyl group, undecyl group, dodecyl group, tridecyl group, tetradecyl group, pentadecyl group, hexadecyl group, heptadecyl group, and octadecyl group.

In one embodiment, preferred examples of R<sup>4</sup> and R<sup>5</sup> include 3-thiapentyl group, 3-thiahexyl group, 3-thiaheptyl group, 3-thiaoctyl group, 3-thianonyl group, 3-thiadecyl group, 3-thiaundecyl group, 4-thiahexyl group, 3-oxapentyl group, 3-oxaheptyl group, 3-oxaheptadecyl group, 3-oxaundecyl group, 3-oxanonyl group, 3-oxadecyl group, 3-oxaundecyl group, 3-oxadodecyl group, 3-oxatridecyl group, 3-oxatetradecyl group, 3-oxapentadecyl group, 3-oxahexadecyl group, 3-oxaheptadecyl group, 3-oxaheptadecyl group, 3-oxanonadecyl group, 4-oxaheptyl group, 4-oxaheptadecyl group, and 4-oxaoctyl group.

The lubricating oil composition may optionally comprise the component (D). When the lubricating oil composition comprises the component (D), the content of the component (D) in the lubricating oil composition is preferably 0.01 to 0.06 mass %, more preferably 0.02 to 0.06 mass %, further preferably 0.02 to 0.05 mass %, and especially preferably 0.02 to 0.04 mass %, in terms of phosphorus on the basis of the total mass of the composition. The content of the component (D) at the above described upper limit or less can further improve electrical insulation of a fresh oil and the oxidatively deteriorated composition. The content of the component (D) at the above described lower limit or more can improve anti-wear performance.

## &lt;(E) Succinimide Ashless Dispersant&gt;

In one preferred embodiment, the lubricating oil composition may further comprise (E) the succinimide ashless dispersant (hereinafter may be referred to as "component (E)"). As the component (E), a boronated succinimide ashless dispersant may be used, a non-boronated succinimide ashless dispersant may be used, or both may be used in combination. In view of further improving electrical insulation of an oxidatively deteriorated oil, the component (E) preferably comprises a boronated succinimide ashless dispersant.

As the component (E), for example, succinimide having at least one alkyl or alkenyl group in its molecule, or any derivative (modified compound) thereof may be used. Examples of the succinimide having at least one alkyl or alkenyl group in its molecule include any compound represented by the following general formula (5) or (6).



## 12

-continued

(6)



In the general formula (5), R<sup>8</sup> represents a C40-400 alkyl or alkenyl group; and b is an integer of 1 to 5, preferably 2 to 4. The carbon number of R<sup>8</sup> is preferably no less than 60, and preferably no more than 350.

In the general formula (6), R<sup>9</sup> and R<sup>10</sup> each independently represent a C40-400 alkyl or alkenyl group, and may be any combination of different groups; and c is an integer of 0 to 4, preferably 1 to 4, more preferably 1 to 3. The carbon numbers of R<sup>9</sup> and R<sup>10</sup> are preferably no less than 60, and preferably no more than 350.

The carbon numbers of R<sup>8</sup> to R<sup>10</sup> in the general formulae (5) and (6) at the above described lower limits or more make it possible to obtain good solubility in the lubricating base oil. In contrast, the carbon numbers of R<sup>8</sup> to R<sup>10</sup> at the above described upper limits or less can improve low-temperature fluidity of the lubricating oil composition.

The alkyl or alkenyl groups (R<sup>8</sup> to R<sup>10</sup>) in the general formulae (5) and (6) may be linear chain or branched, and preferred examples thereof include branched alkyl groups and branched alkenyl groups derived from oligomers of olefins such as propylene, 1-butene, and isobutene, or from co-oligomers of ethylene and propylene. Among them, a branched alkyl or alkenyl group derived from oligomers of isobutene which are conventionally referred to as polyisobutylene, or a polybutenyl group, is most preferable.

The number average molecular weights of the alkyl or alkenyl groups (R<sup>8</sup> to R<sup>10</sup>) in the general formulae (5) and (6) are preferably 1000 to 3500, and more preferably 800 to 3500.

The succinimide having at least one alkyl or alkenyl group in its molecule includes so-called monotype succinimide represented by the general formula (5) where only an amino group at one terminal of a polyamine chain is imidated, and so-called bistype succinimide represented by the general formula (6) where amino groups at both terminals of a polyamine chain are imidated. The component (E) may comprise either monotype or bistype succinimide, or may comprise both as a mixture. The content of bistype succinimide or any derivative (modified compound) thereof in the component (E) is preferably no less than 50 mass %, and more preferably no less than 70 mass %, on the basis of the total mass of the component (B) (100 mass %).

The method for producing the succinimide having at least one alkyl or alkenyl group in its molecule is not specifically limited. For example, such succinimide may be obtained as a condensation reaction product by: reaction of alkyl- or alkenyl-succinic acid having a C40-400 alkyl or alkenyl group or anhydride thereof, with a polyamine. As the component (E), such a condensation product may be used as it is, or may be converted into a derivative (modified compound) described later to be used. The condensation product of alkyl- or alkenyl-succinic acid or anhydride thereof, and a polyamine may be bistype succinimide where both terminals of a polyamine chain are imidated (see the general formula (6)), may be monotype succinimide where only one terminal of a polyamine chain is imidated (see the

general formula (5)), or may be a mixture thereof. Here, an alkenyl-succinic acid anhydride having a C40-400 alkenyl group may be obtained by reaction of a C40-400 alkene and maleic anhydride, and an alkyl-succinic acid anhydride having a C40-400 alkyl group may be obtained by a catalytic hydrogenation reaction of such an alkenyl-succinic acid anhydride. Examples of an alkene to react with maleic anhydride may include oligomers of olefins and co-oligomers of ethylene and propylene as described above, and may include isobutene oligomers. Examples of a polyamine include diethylenetriamine, triethylenetetramine, tetraethylenepentamine, and pentaethylenhexamine, and any mixtures thereof, and a polyamine raw material comprising at least one selected therefrom may be preferably used. The polyamine raw material may further or optionally comprise ethylenediamine. In view of improvement of the performance of the condensation product or derivative (modified compound) thereof as a dispersant, the content of ethylenediamine in the polyamine raw material is preferably 0 to 10 mass %, and more preferably 0 to 5 mass %, on the basis of the total mass of the polyamine raw material. Succinimide obtained as the condensation reaction product of alkyl- or alkenyl-succinic acid having a C40-400 alkyl or alkenyl group or anhydride thereof, and a mixture of at least two polyamines is a mixture of the compounds of the general formulae (5) or (6) having different values of b or c.

Examples of derivatives (modified compounds) of the foregoing succinimide include:

(i) oxygen-containing organic compound-modified compounds where a part or all of the residual amino and/or imino groups is/are neutralized or amidated by reacting succinimide as described above with a C1-30 monocarboxylic acid such as fatty acids, a C2-30 polycarboxylic acid (such as ethanedioic acid, phthalic acid, trimellitic acid, and pyromellitic acid), an anhydride or ester thereof, a C2-6 alkylene oxide, or a hydroxy(poly)oxyalkylene carbonate;

(ii) boron-modified compounds (boronated succinimide) where a part or all of the residual amino and/or imino groups is/are neutralized or amidated by reacting succinimide as described above with boric acid;

(iii) phosphoric acid-modified compounds where a part or all of the residual amino and/or imino groups is/are neutralized or amidated by reacting succinimide as described above with phosphoric acid;

(iv) sulfur-modified compounds obtained by reacting succinimide as described above with a sulfur compound; and

(v) modified compounds obtained by two or more modifications selected from oxygen-containing organic compound-modification, boron-modification, phosphoric acid-modification, and sulfur-modification, on succinimide as described above. Among the derivatives (modified compounds) (i) to (v), a boron-modified compound (boronated succinimide), may be preferably used.

The weight average molecular weight of (E) the succinimide ashless dispersant is preferably 2000 to 20000, more preferably 3000 to 15000, and in one embodiment, 4000 to 9000. The weight average molecular weight of the component (E) at the above described lower limit or more can further improve electrical insulation of a fresh oil and the oxidatively deteriorated composition. The weight average molecular weight of the component (E) at the above described upper limit or less can further improve electrical insulation of the oxidatively deteriorated composition.

The lubricating oil composition may optionally comprise the component (E). When the lubricating oil composition comprises the component (E), the content of the component (E) in the lubricating oil composition is preferably 1 to 10

mass %, and in one embodiment, 1 to 7 mass %, on the basis of the total mass of the lubricating oil composition. The content of the component (E) at the above described upper limit or less can further improve electrical insulation of a fresh oil and the oxidatively deteriorated composition. The content of the component (E) at the above described lower limit or more can improve electrical insulation of a fresh oil. In view of further improvement of electrical insulation of the oxidatively deteriorated composition, the content of the component (E) in the lubricating oil composition is preferably no more than 0.25 mass % in terms of nitrogen on the basis of the total mass of the lubricating oil composition.

<(F) Antioxidant>

In one preferred embodiment, the lubricating oil composition may further comprise (F) the antioxidant (hereinafter may be referred to as "component (F)"). As the component (F), one compound may be used alone, and at least two compounds may be used in combination. As the component (F), any known antioxidant such as an amine antioxidant and a phenolic antioxidant may be used without particular limitation. As the component (F), at least one amine antioxidant may be used, at least one phenolic antioxidant may be used, or any of them may be used in combination.

Examples of the amine antioxidant include aromatic amine antioxidants and hindered amine antioxidants. As the amine antioxidant, at least one aromatic amine antioxidant may be used, at least one hindered amine antioxidant may be used, or any of them may be used in combination. Examples of the aromatic amine antioxidant include primary aromatic amine compounds such as alkylated- $\alpha$ -naphthylamine; and secondary aromatic amine compounds such as alkylated diphenylamine, phenyl- $\alpha$ -naphthylamine, alkylated phenyl- $\alpha$ -naphthylamine, and phenyl- $\beta$ -naphthylamine. As the aromatic amine antioxidant, alkylated diphenylamine, or alkylated phenyl- $\alpha$ -naphthylamine, or the combination thereof may be preferably used.

Examples of the hindered amine antioxidant include 2,2,6,6-tetraalkylpiperidine derivatives. As the 2,2,6,6-tetraalkylpiperidine derivative, a 2,2,6,6-tetraalkylpiperidine derivative having a substituent in 4-position is preferable. Two 2,2,6,6-tetraalkylpiperidine skeletons may be bonded with each other via a substituent in their respective 4-positions. There may be no substituent in N-position of the 2,2,6,6-tetraalkylpiperidine skeleton, and a C1-4 alkyl group may be substituted in N-position thereof. The 2,2,6,6-tetraalkylpiperidine skeleton is preferably 2,2,6,6-tetramethylpiperidine skeleton.

The substituents in 4-position of the 2,2,6,6-tetraalkylpiperidine skeleton include acyloxy group ( $R^{11}COO-$ ), alkoxy group ( $R^{11}O-$ ), alkylamino group ( $R^{11}NH-$ ), and acylamino group ( $R^{11}CONH-$ ).  $R^{11}$  is preferably a C1-30, more preferably a C1-24, and further preferably a C1-20 hydrocarbon group. Examples of the hydrocarbon group include alkyl group, alkenyl group, cycloalkyl group, alkylcycloalkyl group, aryl group, alkylaryl group, and arylalkyl group.

Examples of the substituents when two 2,2,6,6-tetraalkylpiperidine skeletons are bonded with each other via a substituent in their respective 4-positions include hydrocarbylene bis(acyloxy) group ( $-OOC-R^{12}-COO-$ ), hydrocarbylene diamino group ( $-HN-R^{12}-NH-$ ), and hydrocarbylene bis(carbonylamino) group ( $-HNCO-R^{12}-CONH-$ ).  $R^{12}$  is preferably a C1-30 hydrocarbylene group, which is more preferably an alkylene group.

An acyloxy group is preferable as a substituent in 4-position of the skeleton of 2,2,6,6-tetraalkylpiperidine. One example of compounds having an acyloxy group in 4-posi-

tion of the 2,2,6,6-tetraalkylpiperidine skeleton is an ester of 2,2,6,6-tetramethyl-4-piperidinol and a carboxylic acid. Examples of such a carboxylic acid include C8-20 linear or branched chain aliphatic carboxylic acids.

Examples of the phenolic antioxidant include 4,4'-methylenebis(2,6-di-tert-butylphenol); 4,4'-bis(2,6-di-tert-butylphenol); 4,4'-bis(2-methyl-6-tert-butylphenol); 2,2'-methylenebis(4-ethyl-6-tert-butylphenol); 2,2'-methylenebis(4-methyl-6-tert-butylphenol); 4,4'-butylidenebis(3-methyl-6-tert-butylphenol); 2,2'-isopropylidenebis(2,6-di-tert-butylphenol); 2,2'-methylenebis(4-methyl-6-nonylphenol); 2,2'-isobutylidenebis(4,6-dimethylphenol); 2,2'-methylenebis(4-methyl-6-cyclohexylphenol); 2,6-di-tert-butyl-4-methylphenol; 2,6-di-tert-butyl-4-ethylphenol; 2,4-dimethyl-6-tert-butylphenol; 2,6-di-tert-butyl-4-(N,N'-dimethylaminomethyl)phenol; 4,4'-thiobis(2-methyl-6-tert-butylphenol); 4,4'-thiobis(3-methyl-6-tert-butylphenol); 2,2'-thiobis(4-methyl-6-tert-butylphenol); bis(3-methyl-4-hydroxy-5-tert-butylbenzyl) sulfide; bis(3,5-di-tert-butyl-4-hydroxybenzyl) sulfide; 2,2'-thiodiethylene bis[3-(3,5-di-tert-butyl-4-hydroxyphenyl)propionate]; tridecyl-3-(3,5-di-tert-butyl-4-hydroxyphenyl)propionate; pentaerythritol tetrakis[3-(3,5-di-tert-butyl-4-hydroxyphenyl)propionate]; octyl 3-(3,5-di-tert-butyl-4-hydroxyphenyl)propionate; octadecyl 3-(3,5-di-tert-butyl-4-hydroxyphenyl)propionate; and 3-methyl-5-tert-butyl-4-hydroxyphenol fatty acid esters.

The lubricating oil composition may optionally comprise the component (F). When the lubricating oil composition comprises an amine antioxidant as the component (F), the content of the amine antioxidant in the lubricating oil composition is preferably more than 0 mass % and no more than 0.15 mass %, and in one embodiment, may be more than 0 mass % and no more than 0.12 mass %, in terms of nitrogen on the basis of the total mass of the lubricating oil composition. The content of the amine antioxidant at the above described upper limit or less can further improve electrical insulation of a fresh oil and the oxidatively deteriorated composition. The lower limit of the content of the amine antioxidant is not particularly limited, but in one embodiment, may be no less than 0.005 mass % in terms of nitrogen.

When the lubricating oil composition comprises a phenolic antioxidant as the component (F), the content of the phenolic antioxidant in the lubricating oil composition is preferably more than 0 mass % and no more than 1.5 mass %, and in one embodiment, may be more than 0 mass % and no more than 1.0 mass %, on the basis of the total mass of the lubricating oil composition. The content of the phenolic antioxidant at the above described upper limit or less can further improve electrical insulation of a fresh oil and the oxidatively deteriorated composition. The lower limit of the content of the phenolic antioxidant is not particularly limited, but in one embodiment, may be no less than 0.1 mass %.

#### <Other Additives>

In one embodiment, the lubricating oil composition may further comprise at least one additive selected from viscosity index improvers, pour point depressants, anti-wear agents or extreme-pressure agents other than the component (D), friction modifiers other than the component (B), corrosion inhibitors other than the component (A), metal deactivators other than the component (A), anti-rust agents, demulsifiers, anti-foaming agents, and coloring agents.

As the viscosity index improver, any viscosity index improver that is used in lubricating oils may be used without particular limitations. Examples of such a viscosity index

improver include polymethacrylates, ethylene- $\alpha$ -olefin copolymers and hydrogenated products thereof, copolymers of an  $\alpha$ -olefin and an ester monomer having a polymerizable unsaturated bond, polyisobutylene and hydrogenated products thereof, hydrogenated products of styrene-diene copolymers, styrene-maleic anhydride/ester copolymers, and polyalkylstyrene. Among them, a polymethacrylate, an ethylene- $\alpha$ -olefin copolymer or a hydrogenated product thereof, or any combination thereof may be preferably used. 10 The viscosity index improver may be dispersant type, or may be non-dispersant type. In one embodiment, the weight average molecular weight of the viscosity index improver may be, for example, 2000 to 30000. The lubricating oil composition may optionally comprise the viscosity index improver. When the lubricating oil composition comprises the viscosity index improver, the content of the viscosity index improver in the lubricating oil composition is preferably no more than 12 mass %, and more preferably no more than 8 mass %, on the basis of the total mass of the 15 composition. The content of the viscosity index improver at the foregoing upper limit or less can further improve electrical insulation of a fresh oil and the oxidatively deteriorated composition. The lower limit of this content is not particularly limited, but in one embodiment, may be no less than 1 mass %.

As the pour point depressant, for example, any known pour point depressant such as a polymethacrylate polymer may be used without particular limitations. The lubricating oil composition may optionally comprise the pour point depressant. When the lubricating oil composition comprises the pour point depressant, the content of the pour point depressant in the lubricating oil composition is preferably no more than 1 mass %, and more preferably no more than 0.5 mass %, on the basis of the total mass of the composition. 20 The content of the pour point depressant at the above described upper limit or less can further improve electrical insulation of a fresh oil and the oxidatively deteriorated composition. The lower limit of this content is not particularly restricted, but in one embodiment, may be no less than 0.1 mass %.

Examples of the anti-wear agent or extreme-pressure agent other than component (D) include sulfur-containing compounds such as disulfides, sulfurized olefins, sulfurized oils, and dithiocarbamates, and phosphorus-containing anti-wear agents other than the component (D). Examples of the phosphorus-containing anti-wear agent other than the component (D) include phosphoric acid, thiophosphoric acid, dithiophosphoric acid, trithiophosphoric acid, and complete or partial esters thereof; phosphorous acid, thiophosphoric acid, dithiophosphoric acid, trithiophosphoric acid, monoesters thereof, diesters thereof (excluding diesters represented by the general formula (3)), and triesters thereof. The lubricating oil composition may optionally comprise the anti-wear agent other than the component (D). When the 25 lubricating oil composition comprises the anti-wear agent other than the component (D), the content of this anti-wear agent in the lubricating oil composition is preferably no more than 10 mass %, and more preferably no more than 5 mass %, on the basis of the total mass of the composition. The content of this anti-wear agent at the above described upper limit or less can further improve electrical insulation of a fresh oil and the oxidatively deteriorated composition.

The lubricating oil composition may optionally comprise a phosphorus-containing additive other than the component (D). The total phosphorus content in the lubricating oil composition is preferably no more than 0.06 mass % on the basis of the total mass of the composition. The total phos- 30

phorus content in the lubricating oil composition at the above described upper limit or less can further improve electrical insulation of a fresh oil and the oxidatively deteriorated composition. In one embodiment, the total content of the phosphorus-containing additive other than the component (D) in the lubricating oil composition is preferably 0 to 0.05 mass %, and more preferably 0 to 0.03 mass %, in terms of phosphorus on the basis of the total mass of the composition. The total content of the phosphorus-containing additive other than the component (D) at the above described upper limit or less can further improve electrical insulation of a fresh oil and the oxidatively deteriorated composition.

As the friction modifier other than the component (B), for example, at least one friction modifier selected from organic molybdenum compounds and oiliness agent-based friction modifiers other than the component (B) may be used. The lubricating oil composition may optionally comprise the friction modifier other than the component (B). When the lubricating oil composition comprises the friction modifier other than the component (B), the content of this friction modifier in the lubricating oil composition is preferably no more than 1.0 mass %, and more preferably no more than 0.5 mass %, on the basis of the total mass of the composition. The content of this friction modifier at the above described upper limit or less can further improve electrical insulation of a fresh oil and the oxidatively deteriorated composition.

Examples of the organic molybdenum compound include sulfur-containing organic molybdenum compounds, and organic molybdenum compounds which do not contain sulfur as a constituent element. Examples of the sulfur-containing organic molybdenum compound include sulfur-containing organic compounds such as molybdenum dithiocarbamate compounds; molybdenum dithiophosphate compounds; complexes of molybdenum compounds (examples thereof include: molybdenum oxides such as molybdenum dioxide and molybdenum trioxide; molybdenum acids such as orthomolybdic acid, paramolybdic acid, and sulfurized (poly)molybdic acid; molybdic acid salts such as metal salts and ammonium salts of these molybdic acids; molybdenum sulfides such as molybdenum disulfide, molybdenum trisulfide, molybdenum pentasulfide, and molybdenum polysulfide; thiomolybdic acid; metal salts and amine salts of thiomolybdic acid; and molybdenum halides such as molybdenum chloride), and sulfur-containing organic compounds (examples thereof include: alkyl (thio) xanthate, thiadiazole, mercaptothiadiazole, thiocarbonate, tetrahydrocarbylthiuram disulfide, bis(di(thio)hydrocarbyl dithiophosphonate) disulfide, organic (poly)sulfide, and sulfurized ester) or other organic compounds; and sulfur-containing organic molybdenum compounds such as complexes of sulfur-containing molybdenum compounds such as the above described molybdenum sulfides and sulfurized molybdic acids, and alkenylsuccinimide. The organic molybdenum compound may be a mononuclear molybdenum compound, or may be a polynuclear molybdenum compound such as binuclear molybdenum compounds and trinuclear molybdenum compounds. Examples of the organic molybdenum compound which does not contain sulfur as a constituent element include molybdenum-amine complexes, molybdenum-succinimide complexes, molybdenum salts of organic acids, and molybdenum salts of alcohols.

The lubricating oil composition may optionally comprise a metal-containing additive other than the metallic detergent (such as organic molybdenum compounds and zinc dialkyl dithiophosphate). The total content of metal elements in the

lubricating oil composition is preferably no more than 0.03 mass % in terms of metal on the basis of the total mass of the composition. The total content of metal elements in the lubricating oil composition at the above described upper limit or less can further improve electrical insulation of a fresh oil and the oxidatively deteriorated composition. In one embodiment, the total content of a metal-containing additive other than the metallic detergent in the lubricating oil composition is preferably no more than 0.010 mass %, 10 more preferably no more than 0.0075 mass %, and further preferably no more than 0.0050 mass %, in terms of metal on the basis of the total mass of the composition. The total content of the metal-containing additive other than the metallic detergent at the above described upper limit or less 15 can further improve electrical insulation of a fresh oil and the oxidatively deteriorated composition.

Examples of the oiliness agent-based friction modifier other than the component (B) include compounds such as fatty acid esters, fatty acids, fatty acid metal salts, aliphatic 20 alcohols, and aliphatic ethers. These compounds each preferably have a C10-30 aliphatic hydrocarbyl or aliphatic hydrocarbylcarbonyl group, more preferably a C10-30 alkyl or alkenyl group or a C10-30 alkylcarbonyl or alkenylcarbonyl group, further preferably a C10-30 linear chain alkyl or linear chain alkenyl group or a C10-30 linear chain alkylcarbonyl or linear chain alkenylcarbonyl group.

As the corrosion inhibitor other than the component (A), for example, any known corrosion inhibitor such as thiadiazole compounds and imidazole compounds may be used 30 without particular limitations. The lubricating oil composition may optionally comprise the corrosion inhibitor other than the component (A). When the lubricating oil composition comprises the corrosion inhibitor other than the component (A), the content of this corrosion inhibitor in the lubricating oil composition is preferably no more than 1 mass %, and more preferably no more than 0.5 mass %, on the basis of the total mass of the composition. The content of this corrosion inhibitor at the above described upper limit or less can further improve electrical insulation of a fresh oil and the oxidatively deteriorated composition. The lower limit of the content of this corrosion inhibitor is not particularly restricted, but in one embodiment, may be no less than 0.01 mass %.

As the metal deactivator other than the component (A), 45 for example, any known metal deactivator such as imidazoline, pyrimidine derivatives, alkylthiadiazoles, mercapto-benzothiazoles, 1,3,4-thiadiazole polysulfide, 1,3,4-thiadiazolyl-2,5-bis(dialkyl dithiocarbamate), 2-(alkyldithio) benzimidazole, and  $\beta$ -(*o*-carboxybenzylthio)propionitrile 50 may be used without particular limitations. The lubricating oil composition may optionally comprise the metal deactivator other than the component (A). When the lubricating oil composition comprises the metal deactivator other than the component (A), the content of this metal deactivator in the lubricating oil composition is preferably no more than 1 mass %, and more preferably no more than 0.5 mass %, on the basis of the total mass of the composition. The content of this metal deactivator at the above described upper limit or less can further improve electrical insulation of a fresh oil 55 and the oxidatively deteriorated composition. The lower limit of the content of this metal deactivator is not particularly restricted, but in one embodiment, may be no less than 0.01 mass %.

As the anti-rust agent, for example, any known anti-rust 60 agent such as petroleum sulfonate, alkylbenzenesulfonate, dinonylnaphthalenesulfonate, alkenylsuccinate esters, and polyol esters may be used without particular limitations. The

lubricating oil composition may optionally comprise the anti-rust agent. When the lubricating oil composition comprises the anti-rust agent, the content of this anti-rust agent in the lubricating oil composition is preferably no more than 1 mass %, and more preferably no more than 0.5 mass %, on the basis of the total mass of the composition. The content of this anti-rust agent at the above described upper limit or less can further improve electrical insulation of a fresh oil and the oxidatively deteriorated composition. The lower limit of the content of this anti-rust agent is not particularly restricted, but in one embodiment, may be no less than 0.01 mass %. In the present description, the content of any metal sulfonate shall contribute to the content of the metallic detergent even when used as the anti-rust agent.

As the demulsifier, for example, any known demulsifier such as polyoxyalkylene glycol-based nonionic surfactants including polyoxyethylene alkyl ether, polyoxyethylene alkylphenyl ether, and polyoxyethylene alkylnaphthyl ether may be used without particular limitations. The lubricating oil composition may optionally comprise the demulsifier. When the lubricating oil composition comprises the demulsifier, the content of this demulsifier in the lubricating oil composition is preferably no more than 5 mass %, and more preferably no more than 3 mass %, on the basis of the total mass of the composition. The content of this demulsifier at the above described upper limit or less can further improve electrical insulation of a fresh oil and the oxidatively deteriorated composition. The lower limit of this content is not particularly restricted, but in one embodiment, may be no less than 1 mass %.

As the anti-foaming agent, any known anti-foaming agent such as silicones, fluorosilicones, and fluoroalkyl ethers may be used. The lubricating oil composition may optionally comprise the anti-foaming agent. When the lubricating oil composition comprises the anti-foaming agent, the content of this anti-foaming agent in the lubricating oil composition is preferably no more than 0.5 mass %, and more preferably no more than 0.1 mass %, on the basis of the total mass of the composition. The content of this anti-foaming agent at the above described upper limit or less can further improve electrical insulation of a fresh oil and the oxidatively deteriorated composition. The lower limit of this content is not particularly restricted, but in one embodiment, may be no less than 0.0001 mass %.

As the coloring agent, for example, any known coloring agent such as azo compounds may be used.

*<Lubricating Oil Composition>*

The kinematic viscosity of the lubricating oil composition at 100° C. is preferably 1.8 to 4.0 mm<sup>2</sup>/s. The kinematic viscosity of the composition at 100° C. at the above described upper limit or less can improve fuel efficiency. The kinematic viscosity of the composition at 100° C. at the above described lower limit or more can further improve anti-seizure performance, anti-wear performance, anti-fatigue performance, and electrical insulation of a fresh oil and the oxidatively deteriorated composition.

The kinematic viscosity of the lubricating oil composition at 40° C. is preferably 4 to 20 mm<sup>2</sup>/s. The kinematic viscosity of the composition at 40° C. at the above described upper limit or less can improve fuel efficiency. The kinematic viscosity of the composition at 40° C. at the above described lower limit or more can further improve anti-seizure performance, anti-wear performance, anti-fatigue performance, and electrical insulation of a fresh oil and the oxidatively deteriorated composition.

In one embodiment, the volume resistivity of an oxidatively deteriorated oil of the lubricating oil composition at

80° C. is preferably no less than 1.0×10<sup>9</sup> Ω·cm. In the present description, the volume resistivity of an oxidatively deteriorated oil is volume resistivity of an oxidatively deteriorated oil measured at 80° C. in oil temperature, conforming to the volume resistivity test specified in JIS C2101: this oxidatively deteriorated oil is obtained by oxidation treatment on a fresh oil at 165° C. for 150 hours by the ISOT method (Indiana Stirring Oxidation Test) specified in JIS K2514-1.

10 In one embodiment, the total content of any compound having a non-phenolic OH group (which may be part of any other functional group (such as carboxy group and phosphoric acid group)) or a salt thereof, >NH group, or —NH<sub>2</sub> group (hereinafter may be referred to as “O/N-based active hydrogen-containing group”), and not contributing to any content of the metallic detergent, the succinimide ashless dispersant, the amine antioxidant, the component (B1), a phosphite diester compound that does not have an O/N-based active hydrogen-containing group in its alcohol residue (such as the component (D)), and the tolyltriazole metal deactivator is preferably 0 to 500 mass ppm, in one embodiment, 0 to 300 mass ppm, and in another embodiment, 0 to 150 mass ppm, on the basis of the total mass of the lubricating oil composition in terms of the sum of the oxygen element content and the nitrogen element content. Examples of such an O/N-based active hydrogen compound include phosphoric acid (which may be in a form of a salt) and partial esters thereof; phosphorous acid (which may be in a form of a salt) and partial esters thereof (it is noted that 15 any phosphite diester compound that does not have the above described O/N-based active hydrogen-containing group in its alcohol residue shall not fall under the O/N-based active hydrogen compound); nitrogen-containing oiliness agent-based friction modifiers each having a N—H bond (such as primary fatty amines, secondary fatty amines, fatty acid primary amides, fatty acid secondary amides, aliphatic ureas each having a N—H bond, and fatty acid hydrazides); nitrogen-containing oiliness agent-based friction modifiers each having a hydroxy group (such as amides of fatty acids and primary or secondary alkanolamines, and amides of primary or secondary fatty amines and aliphatic hydroxy acids); nitrogen-containing oiliness agent-based friction modifiers each having a carboxy group (which may be in a form of a salt) (such as N-acylated amino acids); oiliness agent-based friction modifiers each having a hydroxy group (such as glycerol monooleate), and oiliness agent-based friction modifiers each having a carboxy group (which may be in a form of a salt) (such as fatty acids and fatty acid metal salts). When one O/N-based active hydrogen compound comprises both an oxygen element and a nitrogen element, the amounts of both an oxygen element and a nitrogen element derived from this compound shall contribute to the total content of the O/N-based active hydrogen compound (total amount of oxygen and nitrogen elements) 20 irrespective of whether each oxygen atom of the compound is bonded to a hydrogen atom and irrespective of whether each nitrogen atom of the compound is bonded to a hydrogen atom. The total content of the O/N-based active hydrogen compound at the above described upper limit or less can further improve electrical insulation of a fresh oil and the oxidatively deteriorated oil.

(Use)

The lubricating oil composition according to the present invention has improved long-term stability of electrical insulation and copper corrosion inhibition performance after oxidatively deteriorated, and thus may be preferably used as an electric motor oil, a transmission oil, a common lubri-

cating oil for electric motors and transmissions (gear mechanisms), or a lubricating oil for electric drive modules including an electric motor and a transmission (gear mechanism). In one embodiment, the lubricating oil composition according to the present invention may be preferably used for lubrication of electric motors in automobiles including the electric motor. In another embodiment, the lubricating oil composition according to the present invention may be preferably used for lubrication of electric motors and transmissions (gear mechanism) in automobiles including the electric motor and the transmission (gear mechanism).

## EXAMPLES

Hereinafter, the present invention will be further specifically described based on examples and comparative examples. The present invention is not limited to these examples.

Examples 1 to 18 and Comparative Examples 1 to 3

As shown in tables 1 to 4, lubricating oil compositions according to the present invention (examples 1 to 18), and lubricating oil compositions for comparison (comparative examples 1 to 3) were each prepared. In the tables, "mass %" for the base oil means mass % on the basis of the total mass of the base oils (the total mass of the base oils is defined as 100 mass %), "mass %" for the other components means mass % on the basis of the total mass of the composition (the total mass of the composition is defined as 100 mass %), and "mass ppm" for the other components means mass ppm on the basis of the total mass of the composition. Details of the components are as follows.

## (Lubricating Base Oil)

O-1: hydrorefined mineral oil (Group II, kinematic viscosity (40° C.): 7.7 mm<sup>2</sup>/s, kinematic viscosity (100° C.): 2.3 mm<sup>2</sup>/s, viscosity index: 118, sulfur content: less than 1 mass ppm)

O-2: hydrorefined mineral oil (Group III, kinematic viscosity (40° C.): 19.5 mm<sup>2</sup>/s, kinematic viscosity (100° C.): 4.2 mm<sup>2</sup>/s, viscosity index: 125, sulfur content: less than 1 mass ppm)

O-3: wax isomerized base oil (Group III, kinematic viscosity (40° C.): 9.3 mm<sup>2</sup>/s, kinematic viscosity (100° C.): 2.7 mm<sup>2</sup>/s, viscosity index: 125, sulfur content: less than 1 mass ppm)

O-4: wax isomerized base oil (Group III, kinematic viscosity (40° C.): 15.7 mm<sup>2</sup>/s, kinematic viscosity (100° C.): 3.8 mm<sup>2</sup>/s, viscosity index: 143, sulfur content: less than 1 mass ppm)

O-5: poly- $\alpha$ -olefin (Group IV, kinematic viscosity (40° C.): 5.0 mm<sup>2</sup>/s, kinematic viscosity (100° C.): 1.7 mm<sup>2</sup>/s)

O-6: poly- $\alpha$ -olefin (Group IV, kinematic viscosity (40° C.): 18.4 mm<sup>2</sup>/s, kinematic viscosity (100° C.): 4.1 mm<sup>2</sup>/s, viscosity index: 124)

O-7: monoester base oil (Group V, kinematic viscosity (40° C.): 8.5 mm<sup>2</sup>/s, kinematic viscosity (100° C.): 2.7 mm<sup>2</sup>/s, viscosity index: 177)

20 ((A) Triazole Metal Deactivator)

A-1: tolyltriazole metal deactivator

A-2: benzotriazole metal deactivator

((B) Succinimide Friction Modifier)

B-1: succinimide compound represented by the general formula (1) (in the general formula (1), R<sup>1</sup> and R<sup>2</sup> are each an octadecenyl group)

25 B-2\*: polyisobutylene succinimide (in the general formula (1), R<sup>1</sup> and R<sup>2</sup> are each a polyisobutylene group, average carbon number of the polyisobutylene group: 192.8)

((C) Calcium Detergent)

C-1: calcium salicylate detergent, base number: 325 mgKOH/g

((D) Phosphite Ester)

D-1: bis(3-thiaundecyl) hydrogen phosphite

30 <(E) Succinimide Ashless Dispersant>

E-1: boronated succinimide ashless dispersant (weight average molecular weight: 9000)

((F) Antioxidant)

F-1: aromatic amine antioxidant

F-2: phenolic antioxidant

TABLE 1

|                                 | examples           |       |       |       |       |       |
|---------------------------------|--------------------|-------|-------|-------|-------|-------|
|                                 | 1                  | 2     | 3     | 4     | 5     | 6     |
| base oil composition            |                    |       |       |       |       |       |
| O-1                             | mass %             | 85    | 60    | —     | —     | 75    |
| O-2                             | mass %             | 15    | —     | 50    | —     | 15    |
| O-3                             | mass %             | —     | 40    | —     | —     | —     |
| O-4                             | mass %             | —     | —     | —     | 55    | —     |
| O-5                             | mass %             | —     | —     | 50    | 45    | 50    |
| O-6                             | mass %             | —     | —     | —     | —     | 50    |
| O-7                             | mass %             | —     | —     | —     | —     | 10    |
| kinematic viscosity of base oil |                    |       |       |       |       |       |
| 40° C.                          | mm <sup>2</sup> /s | 8.7   | 8.6   | 9.1   | 8.9   | 8.9   |
| 100° C.                         | mm <sup>2</sup> /s | 2.5   | 2.5   | 2.5   | 2.5   | 2.5   |
| (A) metal deactivator           |                    |       |       |       |       |       |
| A-1                             | mass % (N)         | 0.02  | 0.02  | 0.02  | 0.02  | 0.02  |
| A-2                             | —                  | —     | —     | —     | —     | —     |
| (B) friction modifier           |                    |       |       |       |       |       |
| B-1                             | mass % (N)         | 0.001 | 0.001 | 0.001 | 0.001 | 0.001 |
| B-2 *                           | mass % (N)         | —     | —     | —     | —     | —     |

TABLE 1-continued

|                                    |                         | examples |      |      |      |      |      |
|------------------------------------|-------------------------|----------|------|------|------|------|------|
|                                    |                         | 1        | 2    | 3    | 4    | 5    | 6    |
| (C) Ca detergent                   |                         |          |      |      |      |      |      |
| C-1                                | mass % (Ca)             | 0.02     | 0.02 | 0.02 | 0.02 | 0.02 | 0.02 |
| (D) phosphite ester                |                         |          |      |      |      |      |      |
| D-1                                | mass % (P)              | 0.04     | 0.04 | 0.04 | 0.04 | 0.04 | 0.04 |
| (E) ashless dispersant             |                         |          |      |      |      |      |      |
| E-1                                | mass %                  | 7.0      | 7.0  | 7.0  | 7.0  | 7.0  | 7.0  |
| (F) antioxidant                    |                         |          |      |      |      |      |      |
| F-1                                | mass % (N)              | 0.02     | 0.02 | 0.02 | 0.02 | 0.02 | 0.02 |
| F-2                                | mass %                  | 0.5      | 0.5  | 0.5  | 0.5  | 0.5  | 0.5  |
| kinematic viscosity of composition |                         |          |      |      |      |      |      |
| 40° C.                             | mm <sup>2</sup> /s      | 9.7      | 9.1  | 10.5 | 10.1 | 10.2 | 9.6  |
| 100° C.                            | mm <sup>2</sup> /s      | 2.7      | 2.6  | 2.8  | 2.8  | 2.8  | 2.7  |
| viscosity index                    |                         |          |      |      |      |      |      |
| Cu solubility test (150° C., 96 h) |                         | 131      | 121  | 114  | 125  | 116  | 116  |
| Cu concentration                   |                         |          |      |      |      |      |      |
| fresh oil                          | mass ppm                | 20       | 20   | 19   | 20   | 21   | 19   |
| after 150 h standing               | mass ppm                | 20       | 20   | 20   | 19   | 21   | 20   |
| at ambient temp.                   |                         |          |      |      |      |      |      |
| volume resistivity (80° C.)        |                         |          |      |      |      |      |      |
| fresh oil                          | 10 <sup>10</sup> Ω · cm | 0.34     | 0.34 | 0.34 | 0.34 | 0.34 | 0.35 |
| oxidatively deteriorated oil       | 10 <sup>10</sup> Ω · cm | 0.21     | 0.21 | 0.21 | 0.21 | 0.21 | 0.20 |

TABLE 2

|                                 |                    | examples |       |       |       |       |       |
|---------------------------------|--------------------|----------|-------|-------|-------|-------|-------|
|                                 |                    | 7        | 8     | 9     | 10    | 11    | 12    |
| base oil composition            |                    |          |       |       |       |       |       |
| O-1                             | mass %             | —        | 50    | 27    | 85    | 85    | 85    |
| O-2                             | mass %             | —        | 50    | 73    | 15    | 15    | 15    |
| O-3                             | mass %             | —        | —     | —     | —     | —     | —     |
| O-4                             | mass %             | —        | —     | —     | —     | —     | —     |
| O-5                             | mass %             | 100      | —     | —     | —     | —     | —     |
| O-6                             | mass %             | —        | —     | —     | —     | —     | —     |
| O-7                             | mass %             | —        | —     | —     | —     | —     | —     |
| kinematic viscosity of base oil |                    |          |       |       |       |       |       |
| 40° C.                          | mm <sup>2</sup> /s | 5.0      | 11.8  | 14.7  | 8.7   | 8.7   | 8.7   |
| 100° C.                         | mm <sup>2</sup> /s | 1.7      | 3.0   | 3.5   | 2.5   | 2.5   | 2.5   |
| (A) metal deactivator           |                    |          |       |       |       |       |       |
| A-1                             | mass % (N)         | 0.02     | 0.02  | 0.02  | 0.005 | 0.03  | —     |
| A-2                             | mass % (N)         | —        | —     | —     | —     | —     | 0.02  |
| (B) friction modifier           |                    |          |       |       |       |       |       |
| B-1                             | mass % (N)         | 0.001    | 0.001 | 0.001 | 0.001 | 0.001 | 0.001 |
| B-2 *                           | mass % (N)         | —        | —     | —     | —     | —     | —     |
| (C) Ca detergent                |                    |          |       |       |       |       |       |
| C-1                             | mass % (Ca)        | 0.02     | 0.02  | 0.02  | 0.02  | 0.02  | 0.02  |
| (D) phosphite ester             |                    |          |       |       |       |       |       |
| D-1                             | mass % (P)         | 0.04     | 0.04  | 0.04  | 0.04  | 0.04  | 0.04  |
| (E) ashless dispersant          |                    |          |       |       |       |       |       |
| E-1                             | mass %             | 7.0      | 7.0   | 7.0   | 7.0   | 7.0   | 7.0   |
| (F) antioxidant                 |                    |          |       |       |       |       |       |
| F-1                             | mass % (N)         | 0.02     | 0.02  | 0.02  | 0.02  | 0.02  | 0.02  |
| F-2                             | mass %             | 0.5      | 0.5   | 0.5   | 0.5   | 0.5   | 0.5   |

TABLE 2-continued

|                                           |                         | examples |      |      |      |      |      |
|-------------------------------------------|-------------------------|----------|------|------|------|------|------|
|                                           |                         | 7        | 8    | 9    | 10   | 11   | 12   |
| <u>kinematic viscosity of composition</u> |                         |          |      |      |      |      |      |
| 40° C.                                    | mm <sup>2</sup> /s      | 5.7      | 13.1 | 16.1 | 9.7  | 9.7  | 9.7  |
| 100° C.                                   | mm <sup>2</sup> /s      | 1.9      | 3.3  | 3.8  | 2.7  | 2.7  | 2.7  |
| viscosity index                           |                         | 114      | 124  | 126  | 131  | 131  | 131  |
| Cu solubility test (150° C., 96 h)        |                         |          |      |      |      |      |      |
| Cu concentration                          |                         |          |      |      |      |      |      |
| fresh oil                                 | mass ppm                | 20       | 18   | 19   | 20   | 20   | 20   |
| after 150 h standing                      | mass ppm                | 19       | 19   | 20   | 22   | 17   | 21   |
| at ambient temp.                          |                         |          |      |      |      |      |      |
| <u>volume resistivity (80° C.)</u>        |                         |          |      |      |      |      |      |
| fresh oil                                 | 10 <sup>10</sup> Ω · cm | 0.27     | 0.40 | 0.45 | 0.34 | 0.32 | 0.33 |
| oxidatively deteriorated oil              | 10 <sup>10</sup> Ω · cm | 0.15     | 0.27 | 0.31 | 0.22 | 0.19 | 0.22 |

TABLE 3

|                                           |                         | examples |       |       |       |       |       |
|-------------------------------------------|-------------------------|----------|-------|-------|-------|-------|-------|
|                                           |                         | 13       | 14    | 15    | 16    | 17    | 18    |
| <u>base oil composition</u>               |                         |          |       |       |       |       |       |
| O-1                                       | mass %                  | 85       | 85    | 85    | 85    | 85    | 85    |
| O-2                                       | mass %                  | 15       | 15    | 15    | 15    | 15    | 15    |
| O-3                                       | mass %                  | —        | —     | —     | —     | —     | —     |
| O-4                                       | mass %                  | —        | —     | —     | —     | —     | —     |
| O-5                                       | mass %                  | —        | —     | —     | —     | —     | —     |
| O-6                                       | mass %                  | —        | —     | —     | —     | —     | —     |
| O-7                                       | mass %                  | —        | —     | —     | —     | —     | —     |
| <u>kinematic viscosity of base oil</u>    |                         |          |       |       |       |       |       |
| 40° C.                                    | mm <sup>2</sup> /s      | 8.7      | 8.7   | 8.7   | 8.7   | 8.7   | 8.7   |
| 100° C.                                   | mm <sup>2</sup> /s      | 2.5      | 2.5   | 2.5   | 2.5   | 2.5   | 2.5   |
| <u>(A) metal deactivator</u>              |                         |          |       |       |       |       |       |
| A-1                                       | mass % (N)              | 0.02     | 0.02  | 0.02  | 0.02  | 0.02  | 0.02  |
| A-2                                       | mass % (N)              | —        | —     | —     | —     | —     | —     |
| <u>(B) friction modifier</u>              |                         |          |       |       |       |       |       |
| B-1                                       | mass % (N)              | 0.001    | 0.001 | 0.010 | 0.020 | 0.001 | 0.001 |
| B-2 *                                     | mass % (N)              | —        | —     | —     | —     | —     | —     |
| <u>(C) Ca detergent</u>                   |                         |          |       |       |       |       |       |
| C-1                                       | mass % (Ca)             | 0.02     | 0.03  | 0.02  | 0.02  | 0.02  | —     |
| <u>(D) phosphite ester</u>                |                         |          |       |       |       |       |       |
| D-1                                       | mass % (P)              | 0.06     | 0.04  | 0.04  | 0.04  | 0.04  | —     |
| <u>(E) ashless dispersant</u>             |                         |          |       |       |       |       |       |
| E-1                                       | mass %                  | 7.0      | 7.0   | 7.0   | 7.0   | —     | —     |
| <u>(F) antioxidant</u>                    |                         |          |       |       |       |       |       |
| F-1                                       | mass % (N)              | 0.02     | 0.02  | 0.02  | 0.02  | —     | —     |
| F-2                                       | mass %                  | 0.5      | 0.5   | 0.5   | 0.5   | —     | —     |
| <u>kinematic viscosity of composition</u> |                         |          |       |       |       |       |       |
| 40° C.                                    | mm <sup>2</sup> /s      | 9.7      | 9.7   | 9.7   | 9.7   | 8.8   | 8.8   |
| 100° C.                                   | mm <sup>2</sup> /s      | 2.7      | 2.7   | 2.7   | 2.7   | 2.5   | 2.5   |
| viscosity index                           |                         | 131      | 131   | 131   | 131   | 111   | 111   |
| Cu solubility test (150° C., 96 h)        |                         |          |       |       |       |       |       |
| Cu concentration                          |                         |          |       |       |       |       |       |
| fresh oil                                 | mass ppm                | 20       | 20    | 20    | 19    | 20    | 20    |
| after 150 h standing                      | mass ppm                | 20       | 20    | 19    | 19    | 20    | 20    |
| at ambient temp.                          |                         |          |       |       |       |       |       |
| <u>volume resistivity (80° C.)</u>        |                         |          |       |       |       |       |       |
| fresh oil                                 | 10 <sup>10</sup> Ω · cm | 0.28     | 0.28  | 0.34  | 0.34  | 0.32  | 0.37  |
| oxidatively deteriorated oil              | 10 <sup>10</sup> Ω · cm | 0.11     | 0.19  | 0.16  | 0.14  | 0.24  | 0.26  |

TABLE 4

|                                    |                         | comparative examples |      |       |
|------------------------------------|-------------------------|----------------------|------|-------|
|                                    |                         | 1                    | 2    | 3     |
| base oil composition               |                         |                      |      |       |
| O-1                                | mass %                  | 85                   | 85   | 85    |
| O-2                                | mass %                  | 15                   | 15   | 15    |
| O-3                                | mass %                  | —                    | —    | —     |
| O-4                                | mass %                  | —                    | —    | —     |
| O-5                                | mass %                  | —                    | —    | —     |
| O-6                                | mass %                  | —                    | —    | —     |
| O-7                                | mass %                  | —                    | —    | —     |
| kinematic viscosity of base oil    |                         |                      |      |       |
| 40° C.                             | mm <sup>2</sup> /s      | 8.7                  | 8.7  | 8.7   |
| 100° C.                            | mm <sup>2</sup> /s      | 2.5                  | 2.5  | 2.5   |
| (A) metal deactivator              |                         |                      |      |       |
| A-1                                | mass % (N)              | 0.02                 | 0.02 | 0.02  |
| A-2                                | mass % (N)              | —                    | —    | —     |
| (B) friction modifier              |                         |                      |      |       |
| B-1                                | mass % (N)              | —                    | —    | 0.030 |
| B-2 *                              | mass % (N)              | 0.02                 | —    | —     |
| (C) Ca detergent                   |                         |                      |      |       |
| C-1                                | mass % (Ca)             | 0.02                 | 0.02 | 0.02  |
| (D) phosphite ester                |                         |                      |      |       |
| D-1                                | mass % (P)              | 0.04                 | 0.04 | 0.04  |
| (E) ashless dispersant             |                         |                      |      |       |
| E-1                                | mass %                  | 7.0                  | 7.0  | 7.0   |
| (F) antioxidant                    |                         |                      |      |       |
| F-1                                | mass % (N)              | 0.02                 | 0.02 | 0.02  |
| F-2                                | mass %                  | 0.5                  | 0.5  | 0.5   |
| kinematic viscosity of composition |                         |                      |      |       |
| 40° C.                             | mm <sup>2</sup> /s      | 9.7                  | 9.7  | 9.7   |
| 100° C.                            | mm <sup>2</sup> /s      | 2.7                  | 2.7  | 2.7   |
| viscosity index                    |                         |                      |      |       |
| 131                                | 131                     | 131                  | 131  | 35    |
| Cu solubility test (150° C., 96 h) |                         |                      |      |       |
| Cu concentration                   |                         |                      |      |       |
| fresh oil                          | mass ppm                | 20                   | 21   | 20    |
| after 150 h standing               | mass ppm                | 53                   | 60   | 17    |
| at ambient temp.                   |                         |                      |      | 40    |
| volume resistivity (80° C.)        |                         |                      |      |       |
| fresh oil                          | 10 <sup>10</sup> Ω · cm | 0.35                 | 0.36 | 0.35  |
| oxidatively deteriorated oil       | 10 <sup>10</sup> Ω · cm | 0.22                 | 0.25 | 0.08  |

## (Copper Solubility Test)

For each of the lubricating oil compositions, copper corrosion inhibition performance of a fresh oil, and copper corrosion inhibition performance of the composition after the composition had been left standing in the air at ambient temperature for 150 hours were evaluated. The fresh oil, or the lubricating oil composition after the fresh oil had been left standing in the air at ambient temperature for 150 hours was used as a sample oil. A copper plate was put in the sample oil, and the sample oil was left standing in a constant temperature bath at 150° C. for 96 hours. Thereafter, the copper concentration in the sample oil was measured by inductively coupled plasma (ICP) emission spectrometry conforming to JPI-5S-44-2011. The results are shown in tables 1-4. In this test, a lower copper concentration measured for the fresh oil means better copper corrosion inhibition performance of the fresh oil, and a lower copper concentration measured for the lubricating oil composition after the composition had been left standing at ambient temperature for 150 hours means better copper corrosion inhibition performance for a long period of time.

## (Volume Resistivity)

The volume resistivity of the fresh oil and an oxidatively deteriorated oil of each of the lubricating oil compositions were measured. The oxidatively deteriorated oil was obtained by oxidation treatment on the fresh oil at 165° C. in oil temperature for 150 hours by the ISOT (Indiana Stirring Oxidation Test) method conforming to JIS K2514-1. The volume resistivity of the fresh oil, and the volume resistivity of the oxidatively deteriorated oil were each measured at 80° C. in oil temperature conforming to the volume resistivity test specified in JIS C2101. The results are shown in tables 1 to 4. In this test, higher volume resistivity at 80° C. means better electrical insulation. The volume resistivity of the oxidatively deteriorated oil at 80° C. in this test is preferably no less than 1.0×10<sup>9</sup> Ω·cm.

## (Evaluation Results)

The lubricating oil compositions of examples 1 to 17 showed good results in long-term stability of copper corrosion inhibition, and electrical insulation of the oxidatively deteriorated oil.

The lubricating oil composition of comparative example 1, which used the succinimide compound not falling under the component (B) (B-2\*) instead of the component (B) (succinimide friction modifier B-1), showed results inferior in long-term stability of copper corrosion inhibition.

The lubricating oil composition of comparative example 2, which did not comprise the component (B), showed results inferior in long-term stability of copper corrosion inhibition.

The lubricating oil composition of comparative example 3, which comprised too high a content of the component (B), showed results inferior in electrical insulation of the oxidatively deteriorated oil.

We claim:

1. A lubricating oil composition comprising:  
a lubricant base oil;  
(A) a triazole metal deactivator in an amount of 0.005 to 0.03 mass % in terms of nitrogen on the basis of the total mass of the composition; and  
(B1) a succinimide compound represented by the following general formula (1) in an amount of 0.0005 to 0.02 mass % in terms of nitrogen on the basis of the total mass of the composition,

wherein when an oxidatively deteriorated oil of the composition is obtained by oxidatively treating the composition for 150 hours by ISOT method conforming to JIS K2514-1, the oxidatively deteriorated oil has a volume resistivity at 80° C. of no less than 1.0×10<sup>9</sup> Ω·cm:



wherein in the general formula (1), R<sup>1</sup> and R<sup>2</sup> each independently represent a hydrogen atom or a C1-36 linear or branched chain alkyl or alkenyl group, and at least one of R<sup>1</sup> and R<sup>2</sup> is a C8-36 linear or branched chain alkyl or alkenyl group, and n represents an integer of 1 to 10.



14. The lubricating oil composition according to claim 13, further comprising:

(D) a phosphite ester compound represented by the following general formula (3) in an amount of 0.01 to 0.06 mass % in terms of phosphorus on the basis of the total mass of the composition: 5



wherein in the general formula (3), R<sup>4</sup> and R<sup>5</sup> are each 15 independently a C1-18 linear chain hydrocarbon group, or a C4-20 group represented by the following general formula (4):



wherein in the general formula (4), R<sup>6</sup> is a C2-17 linear chain hydrocarbon group, and R<sup>7</sup> is a C2-17 linear chain hydrocarbon group, and X<sup>1</sup> is an oxygen atom or a sulfur atom.

15. The lubricating oil composition according to claim 13, 30 wherein the composition has a kinematic viscosity at 100° C. of 1.8 to 4.0 mm<sup>2</sup>/s.

\* \* \* \* \*